

## UNITED STATES PATENT OFFICE.

THEODOR FREUNDORFER AND ROMAN FREUNDORFER, OF MUNICH, GERMANY.

## LIGHT-SENSITIVE ACID-RESISTANT COMPOSITION OF MATTER.

No Drawing.

Application filed November 22, 1921. Serial No. 516,989.

*To all whom it may concern:*

Be it known that we, THEODOR FREUNDORFER and ROMAN FREUNDORFER, citizens of Germany, residing at Munich, Bavaria, 5 Germany, have invented certain new and useful Improvements in Light-Sensitive Acid-Resistant Composition of Matter; and we do hereby declare the following to be a full, clear, and exact description of the invention, such as will enable others skilled in the art to which it appertains to make and use the same.

This invention relates to a light-sensitive acid-resistant composition of matter adapted 15 for application to the metal plates in the process of making etched printing-plates by the photo-mechanical process.

The object of the present invention is attained by making use of the following 20 circumstance: If an ammoniacal solution of shellac is mixed with a bichromate it becomes sensitive and any metal-plates treated with this light-sensitive acid-resistant varnish or coating may be completely etched 25 after printing and developing, without requiring any further operations. At the same time the film has the property that it will not be dissolved by any of the customary plate-cleaning agents.

30 Our varnish or coating may be conveniently prepared as follows:—Dissolve in a water bath 170 grams shellac powder in 700 c. cm. distilled water and 200 c. cm. ammonia of 0.910 specific gravity. Frequent agitation

is desirable, and the powder will be found 35 to be entirely dissolved when the mixture reaches the boiling point. The solution is then cooled and has added thereto 30 c. cm. of a 10% solution of ammonium bichromate. The varnish is then ready for use and may 40 be preserved for from three to four weeks.

In using our varnish, the zinc plate is carefully cleaned with very fine emery dust and slightly roughened in a  $\frac{1}{2}\%$  nitric acid bath, and the varnish applied in the same 45 manner as when fish glue solution is employed. The applied layer should be thick enough so that no rainbow colors appear and that the completed print shows a slight relief. Care should be taken to distribute the 50 varnish absolutely uniformly as inequalities are readily noticeable in the final product. The time of exposure is approximately the same as for fish glue. The plates are developed in a bath of 1000 c. cm. 96% 55 alcohol and 2 gr. methylviolet B B extra concentration. Development is completed in two to three minutes.

Accordingly what is claimed as new and sought to be protected by Letters Patent 60 is the following:

A composition of matter for a light-sensitive film comprising an ammoniacal shellac solution and a soluble bichromate.

In testimony whereof we hereunto affix 65 our signatures.

THEODOR FREUNDÖRFER.  
ROMAN FREUNDÖRFER.